

## UNITED STATES PATENT OFFICE

2,348,359

METHOD OF EXTENDING THE LIFE OF  
ELECTROLYTIC POLISHING BATHSHenry A. Holden Pray, Columbus, Ohio, assignor  
to Battelle Memorial Institute, Columbus, Ohio,  
a corporation of OhioNo Drawing. Application November 4, 1939,  
Serial No. 302,852

6 Claims. (Cl. 204—140)

This invention relates to a method of extending the useful life of electrolytic polishing baths. More particularly, the invention pertains to a method of regenerating spent electrolytic polishing baths comprising as active ingredients mixed sulfuric and phosphoric acids that have become saturated with nickel salts during the operation of said baths.

Reference is made to my application entitled: "Method of extending the life of electrolytic polishing baths," Serial No. 241,948, filed November 23, 1938.

In the polishing of metals by electrolytic processes it is customary to make the metal article to be polished the anode in an electrolytic solution of suitable composition and to pass therethrough a current of sufficient anodic current density for a length of time sufficient to produce the desired degree of polish on the metal. Suitable compositions for polishing baths usually include sulfuric acid as one of the active ingredients, to which phosphoric acid is advantageously added. Hydrofluoric acid, chromic acid, or like acids, may be substituted for phosphoric acid, or, if desired, organic materials such as glycerol, glycerine, and the water soluble glycols, may be added.

After prolonged operation, an electrolytic polishing bath becomes exhausted, i. e., the bath can no longer be effectively used to polish metals. The efficient life of a bath varies greatly, depending upon its composition and on the particular metal or alloy that has been polished therein. One cause of the exhaustion of the electrolytic polishing bath seems to be an accumulation of salts and other products of electrolysis within the bath.

The cost of the bath itself frequently being a substantial proportion of the total cost of the polishing operation, the importance of devising a method for the restoration or regeneration of the bath becomes evident.

My present method is particularly applicable to the regeneration of electrolytic polishing baths containing mixed sulfuric and phosphoric acids as principal active ingredients. When such a bath is used for the polishing of nickel and its alloys, nickel salts and other products of electrolysis accumulate in the bath during the operation of the same. Eventually, when a certain concentration of nickel salts has been reached, the bath no longer operates effectively. According to the present invention, thus exhausted baths may be regenerated by a heat treatment precipitating such accumulated nickel salts as

nickel sulfate in a form suitable for removal by filtration or other means. Sulfuric acid may be added in an amount sufficient to replace the quantity of sulfate removed as nickel sulfate, to build up the sulfuric acid concentration of the bath to optimum operating strength.

It is therefore an important object of the present invention to provide a method for extending the useful life of electrolytic polishing baths by reducing the concentration of accumulated products of the electrolytic action and by restoring to optimum operating strength the active or principal ingredients of the electrolytic polishing baths.

It is another important object of this invention to provide a simple and efficient method for the restoration of exhausted nickel polishing baths comprising sulfuric and phosphoric acids as active ingredients.

It is a further important object of this invention to provide a method of heat treating electrolytic polishing baths comprising as active ingredients sulfuric and phosphoric acids containing nickel salts accumulated during the operation of said baths, to precipitate therefrom said accumulated nickel salts as nickel sulfate in a form suitable for removal by filtration, and to restore said active ingredients to operating efficiency.

Other and further important objects of this invention will become apparent from the following description and appended claims.

I have found that in the electrolytic polishing of nickel or nickel alloys by means of electrolytic baths of the following composition:

|                      | Broad range         | Narrow range         | Preferred range      |
|----------------------|---------------------|----------------------|----------------------|
| 40 Sulfuric acid     | Per cent<br>5 to 85 | Per cent<br>15 to 60 | Per cent<br>15 to 20 |
| Orthophosphoric acid | 5 to 85             | 15 to 70             | 63 to 67             |
| Water                | Not over 50         | Not over 50          | Balance              |

satisfactory polishing results can be obtained so long as the total weight of nickel anodically introduced into said baths is below a limiting value amounting to about 4.5 to about 5.0 per cent, by weight, of said baths. Nickel concentrations above 5.0 per cent indicate the exhaustion of the baths. Unless otherwise specified, all percentages referred to herein will be understood to refer to percentages by weight rather than by volume. Also, references to the acids should be understood to mean the respective acids themselves as represented by their formulae, such as  $H_2SO_4$ .

and  $H_3PO_4$ . The use of percentages by weight rather than by volume and the designation of the respective acids as 100% acids, rather than as commercial strengths, is in accordance with the disclosure in the co-pending abandoned application Serial No. 241,948, filed November 23, 1938.

I have further found that at the usual operating temperature of the hereinabove specified polishing baths, i. e., at about 120° F., precipitation commences in said baths when the nickel content reaches about 2.5 per cent. The precipitation formed is extremely fine-grained, settles very slowly, and can be filtered off only with great difficulty. The composition of this precipitate can not easily be determined analytically, for the precipitate adsorbs free acids from the baths. However, such analytical data as I have been able to obtain indicate said precipitate to be an acid nickel phosphate.

I have also noted that there is a decided increase in the viscosity of said baths on prolonged use which is indicative of yet other changes occurring therein. Possibly there is a transformation of orthophosphoric acid to a poly acid. That these changes, whatever their nature may be, are important factors affecting the operating efficiency of said baths is shown by the fact that reducing the nickel content of exhausted polishing baths to about 2.5 per cent by filtering off nickel salts precipitated therein does not restore the operating efficiency. In other words, the loss of operating efficiency of electrolytic polishing baths on prolonged operation is not due simply to an accumulation of anodically dissolved nickel therein, and is not curable merely by removal of such anodically introduced nickel. The active acid ingredients of the polishing baths are also transformed chemically on prolonged operation into non-efficient forms, which transformation is per se sufficient to render the baths inoperative. The exhaustion of an electrolytic nickel polishing bath is therefore a complex process affecting the bath as a whole.

According to the present invention, spent electrolytic polishing baths comprising sulfuric and phosphoric acids as active ingredients may be regenerated by a heat treatment at an elevated temperature, for instance, at about 180° F. The exact temperature used is not critical. Merely heating a bath to 180° F. and allowing the same to cool to room temperature suffices to restore operating efficiency. Best results have been obtained by heating at about 180° F. for from one to three hours. Higher or lower temperatures may be used for correspondingly shorter or longer periods of time. Preferably the boiling point of the baths being treated is not exceeded, so that the effectiveness of my process is not dependent upon increasing the salt concentration of the bath by evaporation of the solvent. In fact, I prefer not to have any losses by evaporation during the heat treatment step.

Such heat treatments effect the precipitation of nickel salts, suspended and dissolved in said baths, as a lower hydrate of nickel sulfate, probably as monohydrated nickel sulfate, or as a mixture of lower hydrates of nickel sulfate. These lower hydrates are salts which are less soluble in said baths than the nickel salts originally formed by anodic dissolution and are precipitated as large, rapidly settling crystals that can easily be filtered off. The crystal size and rate of settling, as well as completeness of conversion

to lower hydrates of nickel sulfate, depend on the intensity and time of heat treatment. A heat treatment equivalent to the above disclosed treatment at about 180° F. for from one to three hours will reduce the amount of dissolved nickel in solution to about 0.5 to 1.5 per cent, the undissolved nickel being removable by filtration.

Mere heating to 180° F. followed by cooling yields a more easily handled and more rapidly settling precipitate of nickel sulfate, but the resulting sludge has better filtering properties and the amount of nickel retained in the bath is less if the heat treatment at about 180° F. is prolonged for from one to three hours. Slow cooling promotes crystal growth.

Heating, preferably at about 180° F. for from 1 to 3 hours, as disclosed hereinabove also materially reduces the viscosity of the baths, indicating a corresponding transformation of the acid ingredients of said baths. Possibly there is a reversion of a polyphosphoric acid to orthophosphoric acid.

The precipitated nickel sulfate is suitably removed by filtration. First allowing the precipitate to settle facilitates the filtration operation. Additions of active ingredients, in particular sulfuric acid, should be made as required to compensate for losses in acid content due to removal of precipitated nickel salts.

Heating, preferably at about 180° F. for from 1 to 3 hours, such as disclosed hereinabove coupled with settling, filtering, and addition of make-up acid, serves to restore fully the operating efficiency of spent electrolytic polishing baths. After subsequent repeated exhaustion, the baths may again be regenerated. The cycle may be repeated indefinitely. I have, for instance, successfully operated a polishing bath through a sufficient number of such cycles to remove, as nickel sulfate, an amount of anodically dissolved nickel equal to 43 per cent, by weight, of said bath. At the conclusion of said prolonged cyclic operation the bath showed the same efficiency as at the commencement thereof.

Broadly speaking, the principles of the present invention comprise a regenerative heat treatment of exhausted electrolytic polishing baths containing sulfuric and phosphoric acids as active ingredients, to precipitate anodically dissolved nickel salts as a less hydrated form of nickel sulfate and to restore the activity of the acid ingredients of said baths. This heat treatment is effective within a wide range. The heat treatment can also be effectively used in baths containing as active ingredients sulfuric acid either alone or in combination with acids other than phosphoric acid, precipitation of anodically dissolved nickel being effected while reversion of non-active forms of acid ingredients to active forms takes place.

Although it is believed that the nickel sulfate precipitated as a result of the above described heat treatment is largely in the form of the monohydrate, the possibility of other forms being present containing less than 6 molecules of water of hydration is not excluded. By the term "lower hydrates of nickel sulfate," I mean, therefore, to include the monohydrate itself and mixture of hydrated nickel sulfates containing less than 6 molecules of water.

As pointed out, numerous details of this process may be varied through a wide range without departing from the principles of this invention, and I, therefore, do not propose limiting the

patent granted hereon otherwise than necessitated by the appended claims.

I claim as my invention:

1. The method of restoring lost operating efficiency of a used electrolytic polishing bath which contained originally from 15 to 20 per cent sulfuric acid and from 63 to 67 per cent phosphoric acid, by weight, the balance being largely water, and which also contains nickel salts dissolved anodically during use, which method comprises heating said bath to a temperature between about 180° F. and the boiling point of said bath, allowing said bath to cool, and removing precipitated nickel sulfate therefrom.

2. The method of restoring lost operating efficiency of a used electrolytic polishing bath which contained originally from 15 to 20 per cent sulfuric acid and from 63 to 67 per cent phosphoric acid, by weight, the balance being largely water, and which also contains nickel salts dissolved anodically during use, which method comprises heating said bath to about 180° F., allowing said bath to cool, removing precipitated nickel sulfate therefrom, and adding sulfuric acid thereto to restore the sulfuric acid concentration to operating value.

3. The method of restoring lost operating efficiency of an electrolytic polishing bath which contained originally from 15 to 60 per cent sulfuric acid, from 15 to 70 per cent phosphoric acid, by weight, and not over 50 per cent water, and which also contains nickel salts dissolved anodically during use, which method comprises heating said bath to a temperature between about 180° F. and the boiling point of said bath for a time not exceeding three hours, allowing said bath to cool, removing precipitated nickel sulfate

therefrom and adding acid ingredients to replace losses thereof.

4. The method of extending the useful life of a used electrolytic polishing bath consisting essentially of phosphoric and sulfuric acids and water, in which sulfuric acid is an active ingredient and in which anodically dissolved nickel salts are present, which method comprises heating said bath to a sufficiently high temperature between about 180° F. and the boiling point thereof and for a sufficient period of time to effect precipitation of said nickel salts as a lower hydrate of nickel sulfate and to reactivate said bath.

5. The method of extending the useful life of a used electrolytic polishing bath consisting essentially of phosphoric and sulfuric acids and water, in which sulfuric acid is an active ingredient and in which anodically dissolved nickel salts are present, which method comprises heating said bath to between about 180° F. and the boiling point thereof without substantial evaporation to effect precipitation of said nickel salts as a lower hydrate of nickel sulfate and to reactivate said bath, cooling and removing said nickel sulfate.

6. The method of restoring lost operating efficiency of a used aqueous electrolytic polishing bath containing sulfuric and phosphoric acids as active ingredients in which dissolved nickel salts are present, which method comprises heating said bath to at least about 180° F. to reactivate the bath and to convert a portion of the nickel salts present into and precipitate them as a lower hydrate of nickel sulfate, removing the thus precipitated nickel sulfate, and adding sulfuric acid to said bath to replace losses of said acid.

HENRY A. HOLDEN PRAY.